

A. R. EARNSHAW.

ART OF CASTING MOLTEN METAL.

APPLICATION FILED JUNE 12, 1918.

1,323,583.

Patented Dec. 2, 1919.



Inventor

Arthur R. Earnshaw

Witnesses

John C. Bigner  
James H. Bell

By Riley & Paul

Attorneys

# UNITED STATES PATENT OFFICE.

ARTHUR R. EARNSHAW, OF RIVERTON, NEW JERSEY.

## ART OF CASTING MOLTEN METAL.

1,323,583.

Specification of Letters Patent.

Patented Dec. 2, 1919.

Application filed June 12, 1918. Serial No. 239,529.

*To all whom it may concern:*

Be it known that I, ARTHUR R. EARN-  
SHAW, of Riverton, in the county of Bur-  
lington and State of New Jersey, have in-  
5 vented certain new and useful Improve-  
ments in the Art of Casting Molten Metal,  
whereof the following is a specification,  
reference being had to the accompanying  
drawings, which illustrate in vertical sec-  
10 tion an apparatus adapted to carry out my  
invention.

My invention relates particularly to the  
casting of ingots from steel, or steely met-  
als, although it is not limited to that specific  
15 purpose, and the ultimate result to which it  
is addressed is the formation of an ingot or  
body of metal as nearly as possible homo-  
geneous in character, and relatively free  
20 from internal cavities, whether due to the  
presence of blow holes or to the formation  
of "pipes".

The relation of the procedure character-  
istic of my invention, to these ultimate pur-  
poses, will be explained after the invention  
25 itself has been described.

Referring to the drawings, 1, represents  
a container for molten metal, in this in-  
stance, an ordinary ladle having a tap hole  
2, controlled by the plug 3. The mold is  
30 indicated at 4, and may be of any desired  
type. Beneath the tap hole 2, I provide a  
funnel 10, preferably conical, and having its  
axis in line with the center of the tap hole.  
The outlet 11, at the lower extremity of the  
35 funnel is surrounded by a cylindrical apron,  
or shield 12, the exposed surfaces of the  
ladle, funnel and shield being provided with  
refractory linings, as indicated in the cross  
section view.

40 An induction pipe 13, is introduced  
through the side of the funnel 10, near the  
lower extremity thereof, and terminates in a  
downwardly projecting nozzle 14, whose  
axis coincides substantially with the center  
45 of the outlet 11. The upper surface of the  
inwardly projecting portions of the pipe 13,  
and the nozzle, are protected by a refractory  
shield 15.

The pipe 13, communicates with a suit-  
50 able apparatus (not shown) for supplying  
air or gas under pressure, and said pipe is  
also preferably provided with a branch 16,  
communicating with a source of steam sup-  
ply, which may be used under some circum-  
55 stances. The pipe 13, is also provided with  
a drip or trap 17, adjacent to the funnel,

in order to avoid blowing any undesirable  
water or condensation into the system.

In the drawing I have conventionally  
represented the stream of molten metal 60  
flowing from the ladle into the funnel and  
thence to the mold, from which it will be  
seen that said stream, when it impinges  
upon the protective shield 15, of the pipe 13,  
assumes, for the time, a hollow conical form 65  
on its way to the outlet 11, of the funnel,  
the nozzle 14, of the induction pipe 13, be-  
ing located within the hollow of the cone of  
melted metal.

Air under pressure is forced through the 70  
pipe 13, and downwardly through the noz-  
zle 14, into the interior of the descending  
stream of metal and passes therewith  
through the outlet 11. The air blast, re-  
inforced by the expansion effect of heat, 75  
acts in the nature of an atomizer, dispers-  
ing the metal into relatively small drops or  
globules, and thus affording a maximum of  
surface of the metal for contact with the  
air. 80

On the emergence of the stream from the  
outer end of the funnel, some of the metallic  
drops are splashed laterally against the  
shield or apron 12, from which the metal  
descends into the mold still under the ex-  
85 pansive action of the air. The stream of  
metal is thus confined by the funnel-apron  
structure until it leaves the lower end of the  
apron. The dispersion of the main portion  
of the stream of metal continues down-  
90 ward, the air, however, tending to escape  
from the upper portion of the mold and  
hence without necessarily having any large  
percentage carried down into the body of  
metal already in the mold. The effect of 95  
this action of the air is to cool the metal  
uniformly throughout the entire stream in  
its passage from the ladle into the mold, the  
metal being in what may be termed a uni-  
formly divided condition through the ac-  
100 tion of the expanding air blast discharged  
centrally within the descending stream.

By this means the metal may be cooled as  
nearly as may be found advisable to its  
critical temperature of solidification, while 105  
on the way to the mold, so that the solidifica-  
tion in the mold itself can proceed uni-  
formly and with such rapidity as to avoid  
segregation and as to prevent the formation  
of blow holes. Furthermore, for the same 110  
reason, the change of volume in passing  
from the liquid to the congealed condition

is reduced and the formation of pipes in the ingot is minimized.

By this method an ingot homogeneous and uniform in character can be obtained and the necessity for cropping off and discarding a relatively large percentage of the product is avoided. If desired, a blast of steam or aqueous vapor may be supplied through the pipe 16, in connection with the 10 air blast, and instead of air, a cooling gas, of any desired character for reaction with the metal, or metallurgically inert, can be employed.

I recognize that it is not new to introduce 15 air or steam as an incident to the casting of metal and for the same general purposes as that herein described, but, so far as I am aware, the apparatus and methods used for this purpose have differed substantially in 20 mode of operation and effect from those which are characteristic of my invention, in particulars of which the following may be taken as distinctive.

In one type of treatment, the flow of the 25 stream from the ladle into the mold was protracted and the metal was superficially exposed to the action of air in the course of such protracted passage, as for instance, in Letters Patent of the United States No. 30 1,024,722, dated April 30, 1912.

In another type of treatment, a current of air was forced from the top of the mold to the bottom, during the period of pouring, so as to rise through the body of metal in 35 the mold, as for instance, in Letters Patent of the United States No. 974,934, dated November 8, 1910.

In another type, a blast of gas was caused 40 to impinge upon the surface of the metal in the mold, as set forth in Letters Patent of the United States No. 866,497, dated September 17, 1907.

My process differs from these processes 45 and others of the same general character in that I discharge the blast of gas or vapor practically at the central axis of the descending stream of molten metal before it reaches the mold and in such manner as to disperse the metal symmetrically on its way 50 from the ladle to the mold, and thereby I am enabled to effect the desired cooling with great uniformity, and with a very brief exposure to contact with the air, or vapor. I thus obviate excessive oxidation and also 55 avoid the irregular cooling action, which is characteristic of former processes and which is largely due to the inability to make the surface of contact between the cooling agent and the metal large enough to render the

reaction easily controlled and give the maximum efficiency, in the shortest time. 60

In my claims I use the term "gas" as a convenient one to comprehend air, steam, aqueous vapor, or any other desired cooling medium of similar physical character. 65

Having thus described my invention, I claim:

1. The improvement in the art of casting metal which consists in dispersing the molten metal into relatively small globules 70 on its way from the container to the mold, and subjecting it, while thus dispersed, to the action of a gaseous cooling medium.

2. The improvement in the art of casting metal which consists in dispersing the molten metal into relatively small globules 75 while on its way from the container to the mold, subjecting it, while thus dispersed, to the cooling action of a gaseous blast, and permitting escape of the gas from the metal 80 above the level of the latter in the mold.

3. The improvement in the art of casting metal which consists in subjecting the molten metal, on its way from the container to the mold, to a gaseous blast, so as to disperse it into relatively small globules and cool it by the action of the gas on it while 85 thus dispersed.

4. The hereinbefore described improvement in the art of casting metal, which consists in introducing a blast of gas under pressure into the interior of the stream of descending metal during the passage of the latter from the container to the mold, thereby dispersing and cooling the metal with 90 substantial uniformity; restraining the area of dispersion of the metal; and permitting the substantial escape of the gas from the descending stream at a point above the level 95 of the metal collecting in the mold. 100

5. The improvement in the art of casting metal which consists in confining the stream of molten metal during its passage from the container to the mold and introducing a blast of gas under pressure into the stream 105 of metal while so confined, so as to disperse and cool it and cause it to leave the confining means under the expansive action of the gas, permitting escape of the gas from the metal above the level of the latter in the 110 mold.

In testimony whereof, I have hereunto signed my name at Philadelphia, Pennsylvania, this fourth day of June, 1918.

ARTHUR R. EARNSHAW.

Witnesses:

JAMES H. BELL,  
E. L. FULLERTON.